

# United States Patent Office

Naf  
 CrO<sub>3</sub>  
 H<sub>2</sub>O  
 2,883,311  
 Patented Apr. 21, 1959

1

2,883,311

## METHOD AND COMPOSITION FOR TREATING ALUMINUM AND ALUMINUM ALLOYS

David Halpert, Philadelphia, Pa., assignor to Vertol Aircraft Corporation, Morton, Pa., a corporation of Pennsylvania

No Drawing. Application October 1, 1956  
 Serial No. 614,779

6 Claims. (Cl. 134—3)

This invention relates to the surface treatment of aluminum and aluminum base alloys for the removal of oxide films, and more particularly to the composition and method for treating aluminum surfaces so as to maintain a low electrical resistance for a substantial period of time.

Surface cleaning of aluminum and its alloys, for producing and maintaining a smut-free bright surface, is made difficult by the rapid formation of oxide coatings on aluminum when exposed to the atmosphere. It is essential that the deoxidizing solution dissolve away the natural oxide film without attacking the aluminum metal too sharply, which would result in etching or pitting of the surface. This can be done if a uniform reaction takes place between the aluminum and the deoxidizing solution such that the solution acts on all parts of the surface simultaneously and with the same reaction speed.

It is therefore, a primary object of this invention to provide a chemical deoxidizing solution for removing the oxide coatings on aluminum and its alloys wherein the composition agents are readily controllable at the room operating temperature of the solution, and further, wherein the dimensional tolerance losses of the aluminum are positively controlled by the use of an inhibitor.

A further object of the invention is to provide an aluminum deoxidizing solution comprising an aqueous acid solution containing fluorides, chromates or dichromates and nitric acid in certain well defined proportions and ranges of concentration for producing an electrically low resistant surface without excessively removing the aluminum base metal.

Further objects and advantages of the chemical deoxidizing solution will become apparent from the following description.

The term "deoxidizing solution" is used throughout the description in place of "chemical cleaning solution" because it more accurately defines the function of the solution, which is to remove the characteristic oxide coating on aluminum and its alloys.

In general, the composition of the deoxidizing solution consists of relatively high concentrations of nitric acid and fluorides in combination with hexavalent chromium ions. Nitric acid (70% concentrate) is preferably used in an amount within the range of from about 80 to 90 cc. per liter. The fluoride constituent may be introduced in the form of a simple or complex fluoride which is soluble in nitric acid without producing objectionable precipitates with the chromium ions or the aluminum ions that may find their way into the solution by metal dissolution. Sodium fluoride is preferably used for supplying the fluoride ion since it is easily handled and relatively economical. It has been found that the fluoride ion concentration of the deoxidizing solution should be maintained at an amount approximately equivalent to that obtained with 1 to 45 grams of sodium fluoride per liter of solution. Also, by varying the amount of sodium fluoride introduced into solution, it is possible to control the solution pH value, which for best results should be main-

tained within a range of 0.2 to 1.7, the preferred pH range being 0.35 to 0.9.

Chromic acid is a preferred constituent for supplying the hexavalent chromium ion which acts as the inhibitor for the otherwise vigorously reacting mixture of fluorides and nitric acid. The hexavalent chromium ion when properly proportioned with the fluoride ion and the nitric acid, tends to regulate the dissolving action of the deoxidizing solution on the aluminum such that its dimensional losses do not exceed 0.0002" even for an immersion time of approximately 5 minutes in a 60 to 95° F. solution. It was found that the chromium ion concentration should be maintained in an amount approximately equivalent to that obtained with 1 to 400 grams of anhydrous chromic acid per liter of solution.

Thus, the deoxidizing solution of the present invention essentially comprises:

| 20 | Constituent                                              | Propor-<br>tion<br>Range | Preferred |
|----|----------------------------------------------------------|--------------------------|-----------|
|    | Nitric Acid—HNO <sub>3</sub> (70% concentrate) ...cc./l. | 80 to 980                | 330       |
|    | Sodium Fluoride—NaF (anhydrous) .....g./l.               | 1 to 45                  | 15        |
|    | Chromic Acid—CrO <sub>3</sub> (anhydrous) .....g./l.     | 1 to 400                 | 15        |
| 25 | Water—H <sub>2</sub> O .....                             | Balance                  | Balance   |

Prior to the immersion of the aluminum or its alloy in the deoxidizing solution, the surface is preferably cleaned of heavy oil, grease, buffering compounds and dirt by a suitable cleaner such as a vapor degreaser containing trichlorethylene or perchlorethylene. For further removal of any light residual films remaining after vapor degreasing, a mild alkaline cleaner may be used. Though a number of commercial cleaners of this type are available, a suitable cleaner of this general type can be prepared by using 4 ounces of sodium carbonate and 4 ounces of sodium phosphate per gallon of water. This solution is generally used at a temperature of 140 to 180° F. for about 1 to 3 minutes. It should be noted however, that mild alkaline cleaners which function without etching, are not effective in removing the oxide coating on aluminum surfaces and for this purpose the surface to be cleaned is then subjected to a further treatment in the deoxidizing solution of this invention.

When it is desired to prepare the surface for the application of protective or decorative coatings such as those obtained by anodizing or chromatizing or to prepare the surface for the plating thereon of metallic coatings, the aluminum or aluminum alloy piece is immersed in the deoxidizing solution for a period of anywhere from 5 seconds to 5 minutes depending on the thickness of the surface film and previous treatment. The surface thus produced is rather bright and uniform in appearance and not pitted.

55 The deoxidizing solution of the present invention has been found extremely useful in preparing aluminum and its alloys for spot welding. In this connection, it should be noted that successful spot welding of aluminum depends upon obtaining a low electrical surface resistance, usually less than 100 microhms for the mating surfaces, and maintaining this low resistance until such time as the parts are welded. In order to determine the immersion time required to produce a low electrical surface resistance, test strips of aluminum and several of its alloys were immersed in the hereinabove set forth "preferred" deoxidizing solution at temperatures ranging from 60 to 95° F. and for periods of time ranging from 2 seconds to 5 minutes, after which the strips were removed from the solution, thoroughly rinsed in water and dried. The 60 surface resistance of these test strips was then measured by means of an electrical resistance measuring device of the Kelvin Bridge type, and by plotting resistance read-

2,883,311

Patented Apr. 21, 1959

ings against time of immersion, it was noted that a rapid decrease in surface resistance occurs and that a minimum surface resistance is obtained for an immersion time of approximately 5 to 10 seconds. The plotted curve also indicated that for longer immersion times, the surface resistance increases and becomes greater than 100 microhms for immersion times greater than approximately 20 seconds. However, by varying the proportions of the constituents within the disclosed ranges, deoxidizing solutions were obtained by which the surface resistance remained below 100 microhms for immersion periods substantially in excess of 20 seconds.

It was found that the lower the resistance obtained as the result of a 5 to 10 second immersion, the more stable the deoxidized surface was in maintaining its low resistance. For example, the immersion time which produced a low resistance surface having the greatest stability or so-called shelf life for 24S clad aluminum, was determined to be 10 seconds. This low surface resistance, of less than 10 microhms, was maintained for approximately 2 days and after 30 days was only 30 microhms.

It was also found that electrically low resistance surfaces could be obtained and maintained for prolonged periods by using the hereinabove set forth deoxidizing solution with small amounts of copper dissolved therein. The copper was introduced in the form of a soluble salt, such as copper oxide which is compatible with the solution such that the anion will not form precipitates with other solution constituents. The presence of copper ions in the deoxidizing solution may be as much as that obtained with 1 gram of copper oxide per liter of solution, although the preferred concentration is that obtained with approximately 0.3 gram per liter. Excellent results were also obtained with the addition of other metals selected from the group consisting of iron, zinc, magnesium and manganese which were introduced into the solution in quantities similar to that of the copper and in the form of zinc oxide, magnesium oxide and potassium permanganate. It is believed that these added metals plate by immersion on the aluminum and aluminum alloy surfaces to thereby form a protective film which acts as an oxidation inhibitor without affecting the surface resistance.

Having thus described my invention, what I claim is:

1. The process of treating aluminum and its alloys which comprises immersing the metal in an aqueous solution containing 8 to 98% nitric acid (70% concentrate) and containing fluoride and chromate ions in concentrations corresponding to that obtained in a solution containing 1 to 45 grams of sodium fluoride per liter of solu-

tion and 1 to 400 grams of anhydrous chromic acid per liter of solution for a time sufficient to initially reduce the surface resistance of the metal to below 100 microhms, removing the metal from said aqueous solution before the surface resistance again reaches 100 microhms and thereafter rinsing the thus treated metal.

2. A process according to claim 1 in which the aqueous solution contains copper ions in concentrations corresponding to that obtained in a solution containing up to 10 1 gram of copper oxide per liter of solution.

3. A process according to claim 1 in which the aqueous solution contains metals selected from the group consisting of copper, iron, zinc, magnesium and manganese.

4. An aqueous deoxidizing solution consisting of 15 8 to 98% nitric acid (70% concentrate), fluoride and chromate ions in concentrations corresponding to that obtained in a solution containing 1 to 45 grams of sodium fluoride per liter of solution and 1 to 400 grams of anhydrous chromic acid per liter of solution, and copper ions in concentrations corresponding to that obtained in 20 a solution containing up to 1 gram of copper oxide per liter of solution.

5. An aqueous deoxidizing solution consisting of 8 to 25 98% nitric acid (70% concentrate), fluoride and chromate ions in concentrations corresponding to that obtained in a solution containing 1 to 45 grams of sodium fluoride per liter of solution and 1 to 400 grams of anhydrous chromic acid per liter of solution, and metal ions selected from the group consisting of copper, iron, zinc, 30 magnesium and manganese.

6. The process of treating aluminum and its alloys which comprises immersing the metal in an aqueous solution consisting of 8 to 98% nitric acid (70% concentrate) and fluoride and chromate ions in concentrations corresponding to that obtained in a solution containing 1 to 35 45 grams of sodium fluoride per liter of solution and 1 to 400 grams of anhydrous chromic acid per liter of solution for 5 to 20 seconds, removing the metal from said aqueous solution and thereafter rinsing the thus treated metal.

#### References Cited in the file of this patent

##### UNITED STATES PATENTS

|    |           |           |              |
|----|-----------|-----------|--------------|
| 45 | 2,428,749 | De Long   | Oct. 7, 1947 |
|    | 2,598,889 | Caugherty | June 3, 1952 |
|    | 2,705,500 | Deer      | Apr. 5, 1955 |

##### FOREIGN PATENTS

|         |               |               |
|---------|---------------|---------------|
| 726,660 | Great Britain | Mar. 23, 1955 |
|---------|---------------|---------------|